

# United States Patent Office

2,973,317

Patented Feb. 28, 1961

1

2,973,317

## REFINING RAW LUBE OIL STOCK WITH A MILD HYDROGEN TREATMENT FOLLOWED BY SULFURIC ACID

William B. Watson, Park Forest, Ill., assignor to Sinclair Refining Company, New York, N.Y., a corporation of Maine

No Drawing. Filed Feb. 6, 1958, Ser. No. 713,539

2 Claims. (Cl. 208—264)

My invention relates to an improved method for refining petroleum lubricating oils.

Utilizing sulfuric acid to refine raw lubricating oil stocks is well known in the art. In general, the process consists of mixing, either in batch or continuously, sulfuric acid with the oil, allowing the settling of the resultant sludge to produce an acid oil layer, removing the sludge, neutralizing the sulfonic acids and unreacted sulfuric acid present in the acid oil layer with a base material such as sodium hydroxide, potassium hydroxide, ammonium hydroxide, or sodium carbonate in water solution, e.g., 20 percent solution, and water washing to remove excess base and to yield a neutral oil. The amount of acid required depends upon the strength of the acid employed, and the viscosity of the distillate being treated. Acid dosages can vary over a wider range, but, in general, vary from about 5 pounds per barrel of 50 SUS/100° F. (ASTM D 88) distillate to about 50 pounds per barrel of 6,000 SUS/100° F. distillate. Sulfuric acid strength can vary, in general, from about 85 weight percent to 20 weight percent oleum, but 93 to 98 weight percent sulfuric acid is most often employed.

There are numerous modifications for sulfuric acid-treating oils and removing the sludge formed by the acid treatment. However, regardless of these modifications, this process has a major drawback in that a substantial quantity of, for instance, a raw lube fraction is converted to a sludge material of little or no value.

I have now found that, if the raw stock is hydrogenated prior to the sulfuric acid-treating step, higher yields of finished oil are obtained and, in addition, lesser amounts of acid are required in the acid-treating step. By increasing the yield on acid-treating and decreasing the amounts of acid required, the overall costs of my process are considerably less than those of a straight sulfuric acid-treating process.

My process has been found to be particularly effective in the preparation of lubricating oils from distillates of naphthenic base crudes, e.g., Gulf Coast and California crudes. Such crude oils, if they contain wax, are, preferably, dewaxed prior to the hydrogenation step and the acid-treating step, although the dewaxing can follow the hydrogenation operation. This dewaxing can be carried out, for example, by solvent dewaxing using methyl ethyl ketone and toluene as the solvent to achieve oil of below 25° F. pour point (ASTM D 97). The pour point after dewaxing is determined by that required in the finished oil.

The hydrogenation step of my process involves employing a hydrogenation catalyst. Various methods for manufacturing such catalysts have been described in the art, such as in Byrns Patent 2,325,033, and such catalysts generally consist of from about 2 to 5 percent by weight of cobalt oxide and 5 to 15 percent by weight of molybdc oxide, the balance being alumina. Also useful are, for instance, nickel on porcelain, silica or alumina; molybdenum, tungsten, cobalt, nickel oxides and sulfides; and, platinum and palladium on alumina. A preferred cata-

2

lyst is cobalt molybdate supported on alumina prepared by the method of Keith et al. described in copending application Ser. No. 612,892, filed September 28, 1956.

Further, in the hydrogenation step of my process, a temperature of from 550° to 750° F., a pressure of from 400 to 1500 p.s.i.g. and a weight hourly space velocity (weight units of oil per weight unit of catalyst per hour) of from 0.5 to 5.0 are used. The oil is hydrogenated while it is in admixture with from 700 to 5000 standard cubic feet of hydrogen per barrel of oil.

A specific example which illustrates my process and compares it with the known process of acid treating and then neutralizing a charge stock without a prior hydrogenation is as follows:

Two portions of Gulf Coast reduced crude were vacuum distilled to yield distillate portions having the following characteristics:

|                                    |       |
|------------------------------------|-------|
| Gravity, °API (ASTM D 287)         | 19.9  |
| Flash, °F. (ASTM D 92)             | 440   |
| Viscosity, SUS/100° F. (ASTM D 88) | 1594  |
| Viscosity, SUS/210° F. (ASTM D 88) | 81.12 |
| Viscosity index (ASTM D 567)       | 9.9   |
| Pour, °F. (ASTM D 97)              | 5—    |
| Color, NPA (ASTM D 155)            | 8—    |
| Specific dispersion <sup>1</sup>   | 141.9 |
| Aniline point, °C. (ASTM D 611)    | 88.3  |

<sup>1</sup> Reference: The Chemical Constituents of Petroleum, by A. N. Sacheran, page 109, published by Reinhold Publishing Corporation in 1945. G and E lines of mercury were used in refractometer measurements and temperature was 20° C.

The first distillate portion was then hydrogenated with 1500 standard cubic feet of hydrogen per barrel of distillate at a temperature of 700° F. and a pressure of 500 p.s.i.g. by passing it into contact with a cobalt molybdate on alumina catalyst at a weight hourly space velocity of 3.0. The catalyst used analyzed, on an ignited basis, 2.45 weight percent cobalt, 8.53 weight percent molybdc oxide and the remainder alumina.

The weight yield of hydrogenated distillate after being lightly steam stripped was 99.9 percent, and the resulting product had the following characteristics:

|                        |       |
|------------------------|-------|
| Gravity, °API          | 20.7  |
| Flash, °F.             | 410   |
| Viscosity, SUS/100° F. | 1275  |
| Viscosity, SUS/210° F. | 74.97 |
| Pour, °F.              | 0     |
| Color, NPA             | 4½—   |
| Specific dispersion    | 137.0 |
| Aniline point, °C.     | 89.3  |

The steam-stripped, hydrogenated oil was subjected to sulfuric acid treatment. The strength of the acid employed was 98 weight percent and the acid dosage was 16 pounds of acid per barrel of oil. The acid oil mixture was mixed for 45 minutes at a temperature of from 85° to 90° F. It was then allowed to settle for 16 hours and sludge was drawn off. The acid oil mixture was then subjected to an air blow for 2 hours and again allowed to settle for 16 hours. Sludge was again drawn off. The acid oil yield resulting from this operation was 91.5 percent by weight.

The acid oil was then neutralized with 20 weight percent solution of sodium carbonate (soda ash) and water washed until neutral. The neutralized oil was given a light contact at 200° F. with 2 percent by weight Attapulgus clay. Most acid treated oils are given a light earth treatment as a finishing step; however, the earth treatment

is not essential to the process. The characteristics of the acid treated, neutralized, contacted oil were as follows:

|                        |       |
|------------------------|-------|
| Gravity, °API          | 21.3  |
| Flash, °F.             | 425   |
| Viscosity, SUS/100° F. | 1205  |
| Viscosity, SUS/210° F. | 74.47 |
| Viscosity index        | 24.8  |
| Pour, °F.              | 0     |
| Color, NPA             | 2+    |
| Specific dispersion    | 131.4 |
| Aniline point, °C.     | 91.4  |

The second portion of the vacuum distilled Gulf Coast reduced crude oil was acid treated by the same procedure employed for the first portion, but without prior hydrogenation. In this instance, 32 pounds of 98 weight percent sulfuric acid per barrel of distillate were required and the yield of finished oil, i.e., after neutralization, was 86.0 percent by weight. Such finished oil had the following characteristics:

|                        |       |
|------------------------|-------|
| Gravity, °API          | 21.5  |
| Flash, °F.             | 415   |
| Viscosity, SUS/100° F. | 1321  |
| Viscosity, SUS/210° F. | 77.66 |
| Viscosity index        | 25.6  |
| Pour, °F.              | 0     |
| Color, NPA             | 2½—   |
| Specific dispersion    | 131.9 |
| Aniline point, °C.     | 92.3  |

Thus, a comparison of the procedures used on and the products derived from the two portions of Gulf Coast

reduced crude vacuum distillate shows that, although the products are essentially equivalent in degree of refining in terms of viscosity indices, specific dispersions and aniline points, the product of my process of hydrogenating before acid treating and neutralizing required one-half of the acid used in the known process of acid treating and neutralizing. In addition, the yields, when employing my process, were 5.4 percent higher than that of when the old process was employed.

I claim:

1. In the refining of a raw petroleum lubricating oil, the steps consisting essentially of passing the lubricating oil and hydrogen into contact with a hydrogenation catalyst at a temperature within the range from 550° F. to 15 750° F. and at a pressure within the range 400 to 1500 p.s.i.g. to provide a hydrogenated oil and then treating the hydrogenated oil with sulfuric acid to provide an acid oil, said raw lubricating oil being derived from a naphthenic base crude selected from the group consisting of
- 20 Gulf Coast and California crudes.
2. The method of claim 1 wherein said catalyst is cobalt molybdate supported on alumina.

#### References Cited in the file of this patent

#### UNITED STATES PATENTS

|    |           |               |               |
|----|-----------|---------------|---------------|
| 25 | 1,847,623 | Ott           | Mar. 1, 1932  |
|    | 2,692,226 | Smith         | Oct. 19, 1954 |
| 30 | 2,706,167 | Harper et al. | Apr. 12, 1955 |
|    | 2,779,711 | Goretta       | Jan. 29, 1957 |
|    | 2,779,713 | Cole et al.   | Jan. 29, 1957 |